

[54] NICKEL-BASE SUPERALLOY

[75] Inventor: Arthur R. Cox, Lake Park, Fla.

[73] Assignee: United Aircraft Corporation, East Hartford, Conn.

[22] Filed: June 15, 1971

[21] Appl. No.: 153,444

[52] U.S. Cl..... 75/171, 148/32.5

[51] Int. Cl..... C22c 19/00

[58] Field of Search ..... 75/171, 170; 148/32,  
148/32.5

[56] References Cited

UNITED STATES PATENTS

|           |         |                       |        |
|-----------|---------|-----------------------|--------|
| 3,061,426 | 10/1962 | Bieber.....           | 75/171 |
| 3,642,469 | 2/1972  | Ross et al. ....      | 75/171 |
| 3,415,641 | 12/1968 | Ross.....             | 75/171 |
| 3,385,698 | 5/1968  | MacFarlane et al..... | 75/171 |

3,260,505 7/1966 Ver Snyder..... 75/171

Primary Examiner—Richard O. Dean  
Attorney—Richard N. James

[57] ABSTRACT

A cast, precipitation-hardening alloy, applicable to turbine blades and vanes operating in the 1,200°—1,900° F. temperature range, of a nominal composition, by weight, of 9.5 percent chromium, 10 percent cobalt, 2.5 percent molybdenum, 3.7 percent tungsten, 4.2 percent titanium, 5.2 percent aluminum, 1 percent vanadium, 0.015 percent boron, 0.06 percent zirconium, balance nickel.

The invention herein described was made in the course of or under a contract with the Department of the Air Force.

2 Claims, No Drawings

## NICKEL-BASE SUPERALLOY

## BACKGROUND OF THE INVENTION

The present invention relates in general to the cast, precipitation-hardening nickel-base superalloys and, in particular, to such alloys having application to gas turbine engine blades and vanes.

One of the advanced nickel-base superalloys which is utilized in gas turbine engine blading is that described in the patent to Bieber 3,061,426. This alloy, hereinafter identified as Alloy A, has a nominal composition comprising, in percent by weight, 10 chromium, 15 cobalt, 3 molybdenum, 4.5 titanium, 5.5 aluminum, 1 vanadium, 0.17 carbon, 0.015 boron, 0.06 zirconium, balance nickel.

To meet the ever-increasing demands of the engine designer further strength increases in these alloys are required. In particular, increased creep resistance is of fundamental importance. However, despite the knowledge that the addition of patent strengthening elements such as tungsten would possibly impart the desired improvements, it has been found that the above alloy, as constituted, could not be enriched in such elements because the composition would be forced into sigma formation and a consequent unacceptable embrittlement.

## SUMMARY OF THE INVENTION

The present invention contemplates an alloy comprising, in percent by weight, 9-10 chromium, 9.5-10.5 cobalt, 0-5 molybdenum, 1-5 tungsten, 3.5-5.5 titanium, 3-7 aluminum, 0.5-1.5 vanadium, 0.005-0.025 boron, 0.03-0.1 zirconium, 0-0.25 carbon, balance essentially nickel.

A particular preferred embodiment, hereinafter referred to as FA-375, consists essentially of, in percent by weight, 9-10 chromium, 9.5-10.5 cobalt, 2-3 molybdenum, 3.5-4 tungsten, 4-4.5 titanium, 5-5.5 aluminum, 0.7-1.2 vanadium, 0.015-0.025 boron, 0.04-0.08 zirconium, 0-0.20 carbon (0.15-0.20 for polycrystalline form), balance essentially nickel. In addition, the following maximums are maintained, 0.50 iron, 0.20 manganese, 0.01 phosphorous, 0.01 sulfur and 0.2 silicon. A small amount of hafnium, up to 2.5 weight percent, may optionally be added to the alloy.

In addition to polycrystalline castings, the alloy is adapted to directional solidification techniques, including those suggested by VerSnyder U.S. Pat. No. 3,260,505.

## DESCRIPTION OF THE PREFERRED EMBODIMENTS

In alloys of the general type described, the nickel component is used to set the particular crystal lattice, austenite type, or face-centered cubic system from which a strong intermetallic compound can be precipitated. Aluminum and titanium are utilized to provide the strengthening  $\gamma'$  precipitate  $\text{Ni}_3(\text{Al}, \text{Ti})$ . It is generally considered that cobalt acts to stabilize the  $\gamma'$  phase and that vanadium acts as a  $\gamma'$  precipitate strengthener. Carbon provides strength and ductility by precipitation at grain boundaries. Chromium provides corrosion resistance and both molybdenum and tungsten are solid solution strengtheners. Both boron and zirconium appear to provide additional strengthening.

In directional casting and the production of columnar-grain articles, the slow solidification rates associated therewith have revealed, in some instances, evidence of precracked MC-type carbides which may act as failure sites in fatigue. Accordingly, in such processes low carbon contents are preferred. Hafnium, an expensive rare-earth element, has been shown to provide some improvements in alloy castability and has given evidence of improved creep-rupture ductility.

The provision of an alloy with improved creep strength is not achieved merely by the addition of known strengthening elements to a given alloy formation. As previously described, Alloy A to commercial specification chemistry has proven intolerant of the addition of further strengthening elements because such enrichment has led to the formation of the detrimental sigma phase.

The sigma phase is usually identified as an intermetallic compound of topologically close-packed morphology. It precipitates, often in usage, as hard brittle platelets which form the natural sites in the alloy for mechanical weakness. In alloys of the present type, the susceptibility to sigma phase formation has been found to be directly dependent upon the concentrations in solid solution of chromium, cobalt, iron, molybdenum and the like.

In the alloy of the present invention, substantial improvements in creep resistance have been obtained without any evidence of sigma phase precipitation.

Sigma has not, in fact, been observed after engine operation and exposure of the alloy to 1,040 hours at 1,600°F.

A number of alloys were run to a variety of chemistries and varying heat treatments. Each casting was x-rayed to determine soundness and freedom from inclusions, and macro-etched for grain size and uniformity. Both polycrystalline and columnar-grained castings were actually engine tested.

The as-cast microstructure of the polycrystalline FA-375 alloy proved typical of the rich nickel-base superalloys, i.e., a high volume percentage of the secondary  $\gamma'$  phase with associated regions of a eutectic  $\gamma-\gamma'$ . Similarly dispersed, though in low volume percent, were carbides of the MC-type. Gross segregation was not evident.

Initial  $\gamma'$  phase solutioning, as observed by electron microscopy was evident at approximately 2,100°F. and quite apparent by optical microscopy at 2,150°F. Alloy homogenization was readily noticeable as the exposure temperature was raised toward that of melting. Incipient melting and eutectic dissolution began at 2,250°F. and no degeneration of the primary carbides was observed for any exposure.

The effect of heat treatment on the alloys was pronounced and, in most respects, followed basic correlations between microstructure and mechanical properties. Three basic heat treatment cycles were investigated. The first involved partial  $\gamma'$  solutioning (2,200°F/4 hrs.); reprecipitation and  $\gamma'$  overage (2,000°F/4 hrs.) and final precipitation (1,600°F/12 hrs.). The second involved the first and third cycles of the above, i.e., 2,200°F. solutioning and 1,600°F. final precipitation. The third utilized only the latter two cycles — overaging and final precipitation.

The number three cycle was found to produce optimum levels of strength and ductility for the alloy when cast into random polycrystalline form. The number two

cycle was found best when the alloy was directionally solidified. Thus the preferred heat treatment cycle for the equiaxed grain FA-375 alloy contemplates: solution heat treatment at 1,950°-2,000°F in vacuum of dry argon or hydrogen for four hours with subsequent cooling at a rate equivalent to air cool or faster plus precipitation at 1,600°F ± 25°. The preferred heat treatment for the columnar grain FA-375 alloy contemplates: solution heat treatment at 2,175°-2,200°F for 4 hours in same environment as above plus precipitation at 10 1,600°F ± 25°.

In testing, no structural change was observed after 890 hours at 1,400°F. under a continuously applied load of 85,000 p.s.i. After 54 hours at 1,800°F. and 29,000 p.s.i., the only change is phase coalescence 15 aligning in the direction of applied stress. After 1,040 hours at 1,600°F. under a continuously applied load of 40,000 p.s.i., only phase coalescence and annihilation of the fine precipitate was observed. Had the alloy been prone toward sigma formation, this test would have 20 provided opportunity for its presence. However, none was detected.

4  
Table II

| Temp. °F. | Tensile Test Results (Equiaxed Grain) |             |       |
|-----------|---------------------------------------|-------------|-------|
|           | 0.2% YS, p.s.i.                       | UTS, p.s.i. | EL, % |
| RT        | 120,200                               | 137,600     | 6.5   |
| 1400      | 131,200                               | 152,400     | 5.5   |
| 1600      | 105,800                               | 118,500     | 6.0   |
| 1800      | 58,600                                | 75,500      | 7.0   |

Table III

| Temp. °F. | Tensile Test Results (Columnar Grain) |             |       |
|-----------|---------------------------------------|-------------|-------|
|           | 0.2% p.s.i.                           | UTS, p.s.i. | EL, % |
| RT        | 133,000                               | 164,600     | 10.0  |
| 1800      | 64,750                                | 79,800      | 13.7  |

Table IV

| Temp. °F. | Creep-Rupture Test Results<br>(Columnar Grain) |                     |            |                |
|-----------|------------------------------------------------|---------------------|------------|----------------|
|           | Stress<br>p.s.i.                               | Time<br>to 1%, hrs. | Life, hrs. | Final<br>EL, % |
| 1400      | 90,000                                         | 8.1                 | 789.2      | 8.7            |
| 1800      | 29,000                                         | 26.5                | 77.0       | 9.8            |
| 1805      | 23,500                                         | 99.3                | 196.0      | 6.1            |

The results of mechanical testing of the alloy are summarized in the following tables.

35

Table I

| Alloy   | Creep and Creep Rupture (Equiaxed Grain) |                  |                    |            |
|---------|------------------------------------------|------------------|--------------------|------------|
|         | Temp. °F.                                | Stress<br>p.s.i. | Time<br>to 1% hrs. | Life, Hrs. |
| FA-375  | 1400                                     | 85,000           | 374                | 676        |
| Alloy A | 1400                                     | 83,300           | 58                 | 135        |
| FA-375  | 1600                                     | 50,000           | 133                | 338        |
| Alloy A | 1600                                     | 49,600           | 36                 | 180        |
| FA-375  | 1700                                     | 35,000           | 82                 | 215        |
| Alloy A | 1700                                     | 34,300           | 20                 | 62         |
| FA-375  | 1800                                     | 29,000           | 17                 | 53         |
| Alloy A | 1800                                     | 28,400           | 6                  | 40         |
| FA-375  | 1800                                     | 22,000           | 100                | 255        |
| Alloy A | 1800                                     | 21,500           | 42                 | 140        |

Table V

| Temp. °F. | Tensile Test Results                        |         |             |
|-----------|---------------------------------------------|---------|-------------|
|           | Columnar Grain, Carbon less than 200 p.p.m. | 0.2% YS | UTS, p.s.i. |
| RT        | 137,600                                     | 160,100 | 9.0         |
| 1400      | 161,700                                     | 183,100 | 5.0         |
| 1600      | 109,600                                     | 135,700 | 12.5        |
| 1800      | 78,600                                      | 89,900  | 7.5         |
| 2000      | 37,350                                      | 49,800  | 21.0        |

Table VI

| Temp. °F. | Creep-Rupture Test Results              |                  |                     |            |
|-----------|-----------------------------------------|------------------|---------------------|------------|
|           | Columnar Grain, Carbon below 200 p.p.m. | Stress<br>p.s.i. | Time<br>to 1%, hrs. | Life, hrs. |
| 1400      | 90,000                                  | —                | —                   | 1100.0     |
| 1600      | 50,000                                  | 116.0            | 274.2               | 8.2        |
| 1700      | 35,000                                  | 103.7            | 295.9               | 7.3        |
| 1800      | 29,000                                  | 41.0             | 117.8               | 6.2        |
| 1800      | 28,000                                  | —                | 148.1               | —          |
| 1805      | 23,500                                  | 185.8            | 319.2               | 3.5        |

In the foregoing tabular summary it will be noted in particular that the creep and creep-rupture strengths of the alloy of the present invention are vastly superior to those of Alloy A. As directionally solidified, the FA-3-75 alloy is the strongest alloy of this type in its density range. Thus, there has been provided a cast, precipitation hardening nickel-base superalloy having specific utility in gas turbine engine blades and vanes, and incorporation of such blades and vanes in production hardware is currently in process.

Although the invention has been specifically described in detail in connection with specific examples and preferred embodiments, the invention in its broader aspects is not limited thereto, but departures may be made therefrom within the scope of the accompanying claims without departure from the principles of the invention and without sacrificing its chief advantages.

What is claimed is:

1. A cast, precipitation-hardenable nickel-base superalloy characterized by high creep resistance and creep rupture strength which consists essentially of, by weight, 9-10 percent chromium, 9.5-10.5 percent cobalt, 2-3 percent molybdenum, 3.5-4 percent tungsten, 4-4.5 percent titanium, 5-5.5 percent aluminum, 0.7-1.2 percent vanadium, 0.015-0.025 percent boron, 0.04-0.08 percent zirconium, 0-0.20 percent carbon, balance essentially nickel, the superalloy exhibiting long term stability under conditions of high stress at temperatures in excess of 1,650°F.

2. The alloy of claim 1 wherein:

the alloy microstructure as cast is characterized by a columnar grained microstructure aligned substantially in the direction of solidification.

\* \* \* \* \*

20

25

30

35

40

45

50

55

60

65